

# UNITED STATES PATENT OFFICE.

WILLIAM Y. GAMBEE, OF NEW YORK, N. Y., ASSIGNOR TO EUGENE J.  
McGUIRE, OF NEW YORK, N. Y.

## LINING FOR COMBUSTION-FURNACES.

No. 819,696.

Specification of Letters Patent.

Patented May 1, 1906.

Application filed December 11, 1905. Serial No. 291,224.

*To all whom it may concern:*

Be it known that I, WILLIAM Y. GAMBEE, a citizen of the United States, residing in the borough of Bronx, in the city and State of New York, have invented certain new and useful Improvements in Linings for Combustion-Furnaces, of which the following is a specification.

My invention relates to linings for combustion-furnaces, which linings may be either in the form of a plastic material directly laid within the furnace or in the form of fire-brick previously made and adapted to be laid in the usual manner.

It consists of a new composition of matter for this purpose consisting of Portland cement, ground slate, and cinders. The cinders may be in the form of ordinary steam-ashes as they are taken from beneath the grates of boilers or similar furnaces.

The proportion which I have found most advantageous in producing the lining is as follows: one part cement, two parts ground slate, and two parts cinders. It is of course understood that these proportions may be varied within considerable limits without departing from my invention.

I have found in practice that linings for combustion-furnaces made of the above materials and in substantially the proportions

specified are far more durable than ordinary fire-brick or even than fire-brick of the finest quality. In some cases these linings have endured for more than six months in a furnace, where the best quality of Scotch fire-brick burned out in less than three weeks.

What I claim is—

1. A composition of matter for lining combustion-furnaces and the like, composed of cement, ground slate and cinders.

2. A composition of matter for lining combustion-furnaces and the like, composed of cement, ground slate and cinders in the proportion of one part cement, two parts ground slate and two parts cinders.

3. A composition of matter for lining combustion-furnaces and the like, composed of cement, ground slate and cinders in the proportion of one part cement, two parts ground slate and two parts cinders, the cinders being in the form of ashes taken from beneath the grate of an ordinary furnace.

In testimony whereof I have signed this specification in the presence of two subscribing witnesses.

WILLIAM Y. GAMBEE.

Witnesses:

OLIN A. FOSTER,  
GEO. L. COOPER.